

## UNITED STATES PATENT OFFICE

2,466,163

METHOD OF PRODUCING ACID BESSEMER  
STEEL OR THOMAS STEEL LOW IN NITRO-  
GENWilhelm Ekman and Gösta Erik Hildebrand  
Hildebrand, Fagersta, SwedenNo Drawing. Application June 22, 1945, Serial  
No. 601,070. In Sweden July 10, 1944

4 Claims. (Cl. 75—51)

1

There is a clear difference in certain properties between acid Bessemer or Thomas steel produced in a converter (hereinafter called converter steel), on the one hand, and steel produced according to other methods, e. g. Martin-steel, on the other hand. It has appeared from comparative tests that the higher nitrogen content of the converter steel occasions this difference in the properties also in steel with the same chemical analysis of the other constituents. The high nitrogen content depends on the method of production. Of course, a strong absorption of nitrogen takes place in the process as hitherto usually carried out when the air current is pressed through the steel at the blowing. This is clear from nitrogen analyses showing the following values: Martin-steel 0.003–0.007% nitrogen, converter steel 0.010–0.030% nitrogen.

The special properties which the high nitrogen content gives the converter steel over e. g. Martin-steel, are for example: greater strength (about 7 kgs./mm.<sup>2</sup>), higher yield limit, greater ageing liability, and greater hardness and brittleness after cold treatment. The hardening properties are also influenced by the nitrogen content. Under certain circumstances, e. g. in the production of some kinds of tool steel, automatic steel, tubes and railway rails, some of these properties might be desirable. However, as a rule they are not desirable. In the normal production of merchant iron the high nitrogen content of the converter steel is most often detrimental, particularly with regard to the fact that the nitrogen causes a hardness and brittleness of the steel after cold treatment which is greater than of other steel, e. g. Martin-steel, after the same degree of cold treatment; this has appeared to be a great disadvantage for the converter steel, inter alia in cold-drawing of wire and deep-pressing of sheet metal.

However, it has become apparent that a converter steel, produced with a lower nitrogen content than normally, in the way according to this invention does not show the said specific properties but is completely comparable with e. g. a prime Martin-steel.

The problem of lowering the nitrogen content of the converter steel has on a larger technical scale hitherto been solved in such a way that after finished blowing the converter steel has been conveyed to another steel production furnace, generally an open hearth or electric steel furnace, and been subjected to a further refining in the said furnace. Among other things a lowering of the nitrogen content has been obtained in this second step of the duplex process.

It would, of course, be of great economical importance if such a duplex process could be avoided and a steel with low nitrogen content could be produced directly in a converter. Various sug-

gestions of solving this problem have already been made earlier. For example, it has been suggested to effect the blowing with an oxidizing gas mixture with low nitrogen content, or to bring the melt to boil by adding oxidizing matter after finished or almost finished blowing whereby the nitrogen content would be reduced. The nitrogen content of a steel which is in equilibrium with a gas phase, is directly proportional with the square root of the partial pressure of the nitrogen in the gas mixture. In order to prevent or delay the absorption of nitrogen in the steel by changing the composition of the gas phase or simply obtain a lowering of the nitrogen content of the steel from an earlier higher value (denitration) it is, thus, necessary to lower the nitrogen content of the gas mixture. In the gas flowing through the steel in the converter at normal blowing the nitrogen content lies at about 70%. In order to obtain a denitration the average content must be very much lower. At contents between the normal one (about 70%) and the one necessary for the denitration the absorption rate for the nitrogen is reduced more and more with sinking nitrogen content.

As already mentioned, it is known that a low partial pressure for nitrogen in the gas phase can be obtained by influencing the composition of the blast air admitted into the converter prior to the blast contacting the steel, which can be effected e. g. by enriching the blast air with oxygen.

The object of the present invention is to influence the composition of the gas phase not until it has contacted the steel by adding an oxidizing agent, e. g. iron ore, in the converter one or more times in the course of the blowing. However, in order that a denitration or at least a considerable delay of the nitrogen absorption shall be obtained by such addition it is necessary that according to the invention the supply of the blast air or of the blast air gas mixture at least after the addition is arranged in such a way that the blast air passes only through a certain part of the melt whereas the other part is not subjected to the direct influence of the blast air or of the blast air gas mixture.

Several methods of effecting a partial blowing through according to the invention are possible. In a converter provided with the bottom hitherto used this blowing through is obtained by such tilting of the converter that the larger part of the melt lies on the furnace wall and only a smaller part is in contact with the furnace bottom and thus is flowed through by the blast air. It may also be proceeded in such a way that the blast air is admitted only through part of the furnace bottom or through the wall of the furnace.

By addition of oxidizing agent substantially silicon, manganese, carbon and iron and in a

basic method also phosphorus are oxidized. Only in the carbon oxidation the reaction product is a gas, by the supply of which to the gas phase a reduction of the partial pressure of the remaining components, among them that of the nitrogen, can be obtained. It is an advantageous, although not determinant factor of the process that the contents of other substances than carbon and iron are held as low as can be deemed suitable from other points of view. For their reaction products are not included in the gas phase, and thus they do not contribute to lowering the partial pressure of the nitrogen. Particularly in the acid Bessemer method it is moreover desirable, although not necessary, that the contents of these substances are low as thereby the boiling which is a condition for the denitration or the delay of the nitrogen absorption, more quickly gets into working order and its intensity becomes stronger.

At addition of oxidizing agent at normal blowing, i. e. when the blast air flows practically through the whole melt, no denitration is obtained in spite of the addition, possibly only a slight reduction of the nitrogen absorption rate. The explanation of it is that the volume of the carbon monoxide formed per unit of time at the oxidation is slight in comparison with the volume of the blast air admitted to the steel bath during the same time and of the carbon monoxide formed thereof. The lowering of the partial pressure of the nitrogen in the gas phase then becomes too small to considerably influence the nitrogen content of the steel. Consequently, an already known suggestion of lowering the nitrogen content at Thomas blowing by ore addition during the dephosphorizing period does not bring about any considerable lowering of the nitrogen content.

However, when the addition of the oxidizing agent is combined with a partial blowing through according to the invention things are different, for in this case two oxidizing processes which are different but which merge in one another, will take place in the melt. Part of the melt is oxidized by blast air as well as by the specially added oxidizing agent. In another part through which the blast air does not flow, the oxidation is caused substantially by the specially added oxidizing agent. There is, of course, no sharp limit between these parts.

In the first mentioned part of the melt the nitrogen content of the gas phase is relatively high, and there are thus factors existent to render the absorption of nitrogen feasible. In the other part of the melt the gas phase substantially consists of carbon monoxide. Thus denitration can take place in the said phase. In order to obtain low nitrogen contents it should consequently be seen to it that that part of the melt to which no blast air is admitted, is proportionally large. However, the other part in which the blast air passes, must not be too small, either, because in such a case the oxidation rate becomes too low. Moreover, as regards the specially added oxidizing agent its oxidizing influence is reduced if that agitation of the melt which is caused by the blast air fails to come off.

At the use of some oxidizing agents, e. g. iron ore, considerable heat quantities are required for the reduction of the oxidizing agent. This heat

demands can be covered according to earlier known methods, blast air being admitted also above the surface of the bath, i. e. by blowing in an oblique direction or via special tuyers in the furnace walls. This can also be effected by admitting blast air to the steel bath at such a low depth beneath its surface that the oxygen of the blast air has no time to be consumed during the passage through the steel bath. The oxygen which in some of these ways is admitted above the surface of the steel bath, partially combusts the formed carbon monoxide within the converter and gives a sufficient heat quantity for the above-mentioned reduction.

By the method according to the invention a converter steel can be produced which has the same properties as a Martin-steel of the corresponding analysis. At tests made it has been possible to reduce the nitrogen content of the converter steel to such values as are characteristic of normal Martin-steel.

The method according to the invention can, of course, be used with advantage also in such a method in which an oxidizing gas mixture poorer in nitrogen is blown through instead of air.

Having now described our invention, what we claim as new and desire to secure by Letters Patent is:

1. In a method of producing steel by blowing a metal melt in a converter with a continuous blast of a gas containing air but being otherwise free of nitrogen compounds, the steps of adding to the melt in the converter prior to the completion of the blowing, a nitrogen-free oxidizing agent, and then continuing the blowing without interruption, while retaining the entire melt in the converter, in such a manner that the gas flows through part of the melt only so that final oxidation, with simultaneous denitration, is effected by the added oxidizing agent, the part of the melt traversed by the blast gas after addition of the oxidizing agent being proportioned to maintain a sufficient rate of oxidation.

2. A method as claimed in claim 1 in which the blast gas is air.

3. A method as claimed in claim 1 in which the blast gas is an air-gas mixture.

4. A method as claimed in claim 1 in which iron ore is used as an oxidizing agent.

50 WILHELM EKMAN.

55 GÖSTA ERIK HILDEBRAND HILDEBRAND.

#### REFERENCES CITED

The following references are of record in the file of this patent:

#### UNITED STATES PATENTS

| Number       | Name         | Date          |
|--------------|--------------|---------------|
| 51,401       | Bessemer     | Dec. 5, 1865  |
| 60 86,859    | Phillips     | Feb. 9, 1869  |
| 193,551      | Reese        | July 24, 1877 |
| 287,842      | McDonald     | Nov. 6, 1883  |
| 553,875      | Sherk et al. | Feb. 4, 1896  |
| 2,244,385    | Brassert     | June 3, 1941  |
| 65 2,333,654 | Lellep       | Nov. 9, 1943  |
| 2,390,346    | Bayer        | Dec. 4, 1945  |

#### OTHER REFERENCES

The Journal of the Iron and Steel Institute (British) volume CVII, No. I, 1923, pages 665, 666.